

## UNITED STATES PATENT OFFICE

2,340,358

## PROCESS FOR TREATING FABRICS

Howard A. Young, Westfield, N. J., assignor to  
United States Rubber Company, New York,  
N. Y., a corporation of New Jersey

No Drawing. Application June 3, 1943,  
Serial No. 489,540

12 Claims. (Cl. 117—161)

This invention relates to a process for treating fabrics, more particularly to a process for treating fabrics with water-insoluble synthetic resins.

Aqueous dispersions of water-insoluble synthetic resins have been used to treat fabrics in various ways. In some cases the fabrics are saturated with the resin emulsion or dispersion, and the treated fabric dried to leave a resin deposit on the fabric. Such methods of depositing resins on the fabric impart a harsh and boardy feel to the material.

In my prior Patent 2,173,243 there is disclosed a process for gradually depositing particles of treating material, including artificial resins, on fabric by treatment with an aqueous dispersion of the treating material which gradually exhausts the dispersed particles of resin or other material onto the fabric as the fabric is permitted to remain in contact with the dispersion bath. When resin particles are deposited on a fabric by the process of this prior patent, the fabric retains to a great extent the feel and "handle" of an untreated fabric.

The present invention is an improvement over the process of my prior Patent 2,173,243 in that larger particles of water insoluble synthetic resins are deposited from an aqueous medium onto the fabric, which in the case of knitted fabrics, such as stockings, more effectively locks together the filaments of the yarn thus inhibiting snagging and adding durability to the hosiery.

According to the present invention, the fabric is associated with a dilute aqueous bath containing particles of water-insoluble synthetic resin which have been agglomerated from the dispersed state to the form of flocs which are clearly macroscopic and readily separable from the aqueous medium on standing. The water-insoluble resin or dispersion thereof may be compounded as by the addition of modifiers, fillers, vulcanizing or curing ingredients, and other resins. When the colloidal resin particles are agglomerated from the dispersed state to the flocculated state before deposition according to the present invention, the various compounding ingredients for the resin that may also be dispersed in the aqueous medium become agglomerated along with the resin particles into flocs which contain representative proportions of the various compounding ingredients. Hence, there is the additional advantage over the prior art depositions from a colloidal dispersion of a water-insoluble resin containing dispersed compounding ingredients that the flocs of resin as they are

deposited onto the fabric from the agglomerated treating bath of the present invention will inherently contain representative proportions of all the compounding ingredients in the bath, as distinguished from the independent deposition of resin particles and particles of compounding ingredients from a deposition bath in which the resin and compounding materials are individually dispersed in colloidal condition, as in the prior art. The aqueous dispersion of the water-insoluble synthetic resin may be prepared from the solid resin by dispersing the same, with the addition of plasticizers and dispersing agents if desired, in an aqueous medium by means of a colloid mill, or by adding a plasticizer, if desired, and mixing in a hydrophilic colloidal dispersing agent and masticating with additions of water until the resin becomes dispersed in the aqueous medium, as is well known in the art, or 15 the resin itself may be prepared as by condensation or polymerization in an aqueous medium. Various compounding ingredients may be added to the resin before dispersing, or to the dispersion after preparation. Various water-insoluble synthetic resins dispersed in an aqueous medium are available commercially. The water-insoluble resin particles in any aqueous dispersion, once the resin particles are colloidally dispersed in an aqueous medium, may be agglomerated or flocculated from the dispersed condition by the addition of various agglomerating or flocculating agents in the presence of a sufficient amount of protective to prevent the dispersed resin particles from completely coagulating into a coherent lump, but in the presence of insufficient protective to prevent the resin flocs 20 from depositing on the fabric when in contact therewith.

Various methods are known for agglomerating or flocculating the dispersed particles of water-insoluble synthetic resin and various known stabilizers may be used as protectives for the agglomerates. The resin particles may be agglomerated by a process akin to "salting out," as 25 by the addition of relatively large amounts of monovalent salts of strong acids, for example, ammonium sulphate, to an aqueous dispersion of the resin in the presence of a protein, such as gelatin and an additional protective for the agglomerates. The dispersed particles of water-insoluble synthetic resin may be agglomerated 30 by the addition of mildly alkaline salts such as sodium carbonate to an aqueous dispersion of the resin in the presence of a protein, such as gelatin, or in the presence of a cationic soap. The 35

gelatin or cationic soap, which may be the dispersing agent for the dispersed resin particles, may also act as the stabilizer or protective during the flocculation to prevent lump coagulation of the resin. Another method of agglomerating the resin particles is to precipitate a flocculant salt or acid in the dispersion of synthetic resin, as by precipitating a polyvalent metal silicate or silicic acid gel in the protected resin dispersion. A preferred method is by treating the synthetic resin dispersion with a monovalent salt of a strong acid in the presence of both clay and a protein, such as gelatin, and also a protective for the agglomerates.

Various well known protectives or stabilizers may be used to prevent the flocs in the bath from completely coagulating into a coherent mass. The amount of stabilizer necessary to protect the agglomerates will depend on the specific protective used, the method of agglomeration, and the temperature and concentration of the bath, but in any given case may readily be determined empirically. Large excess of stabilizer over that necessary to prevent complete coagulation should be avoided, as the greater the amount of stabilizer added in excess of that needed to prevent complete coagulation, the slower will be the deposition of the resin particles on the fabric. Examples of well known protectives or stabilizers are certain compounds of carboxyl ( $R-COO$ ), sulphonate ( $R-SO_3M$ ), sulphuric ( $R-SO_2M$ ), or phenolic ( $R-OM$ ) groups, or of ethereal sulphuric ( $RO.SO_3M$ ), radicals, where the R may have a straight chain or ring structure, and may contain substituent halogen, amine, nitro or hydroxyl groups, and the M may be an alkali metal, hydrogen or ammonium radical. I have found very satisfactory in the present invention, protectives having the general formula  $R-SO_3M$ , where R represents an organic radical containing at least one group containing more than 8 carbon atoms and M represents alkali metal, hydrogen or ammonium radical. Various commercial stabilizers having this general formula  $R-SO_3M$  are illustrated below with reference to various classifications of the radical R:

(1) Where R is an  $\alpha$ alkoxy group producing, as for example, various compounds from  $C_{10}H_{21}O-SO_3Na$  to  $C_{14}H_{27}O-SO_3Na$ , known commercially under the trade names Gardinol, Duponol, Aquarex D, Orvus WA.

(2) Where R is an alkyl group producing, as for example in the formulae  $C_{12}H_{25}-SO_3Na$  and  $C_{16}H_{33}-SO_3Na$ , lauryl sodium sulphonate and cetyl sodium sulphonate, respectively.

(3) Where R is a mixed ether of long and short chain aliphatic groups, as for example in the compound  $C_{17}H_{33}-O-C_2H_4-SO_3Na$ , believed to be the material known commercially as Nacco-nol LA.

(4) Where R is an alkyl ester of a long chain fatty alcohol, as for example in the compound



known commercially by the trade names Igepon A and Arctic Syntex A.

(5) Where R is a glycol ester of a long chain fatty alcohol, as for example in the formula



(6) Where R is an alkyl substituted amid of a fatty acid, as for example in the compounds



and



10 believed to be the commercial products Igepon T and Igepon TF, respectively.

(7) Where R is an alkyl substituted aromatic radical as in various commercial compounds having the formula



20 as for example, the sodium salts of alkyl naphthalene sulphonic acid, known under the trade names Nekal; Alkanol; a free alkyl naphthalene sulphonic acid, known commercially as Leonil SBS; the potassium salt of an alkyl naphthalene sulphonic acid known under the trade name Eunaphthol K.

25

(8) Where R is a hydroaromatic radical, as for example in the compound



known under the trade name Octaton. Also where R is a hydroaromatic radical as in various commercial compounds having the formula



as for example, where M is sodium as in Alkanol S and Mayamin; where M is potassium as in Mayaminkalium; and where M is ammonium as in Mayammonium.

(9) Where R is an ester of a dibasic acid, such as



in which one of  $R_1$  and  $R_2$  may be an alkyl radical from  $C_3H_7$ — to  $C_8H_{17}$ — and the other hydrogen, or both  $R_1$  and  $R_2$  such as alkyl radical, as for example in the commercial stabilizer known as Aerosol OT which has the formula



The water-insoluble synthetic resin may be of any type to impart the desired properties to the fabric, for example, phenol-aldehyde resins, urea aldehyde resins, melamine-aldehyde resins, aromatic amine-aldehyde resins, synthetic linear organic polyamids (condensation polymerization of a diamine and a dibasic carboxylic acid e. g. hexamethylene diamine and adipic acid), acrylic

resins (polymers or copolymers of the monomeric derivatives, i. e. esters, amides, salts, halides, or nitriles of acrylic acid or methacrylic acid), alkyd resins (polydric alcohol-polybasic acid polymers), polyterpene resins (polymerization of turpentine or copolymerization of turpentine residue and fish oil), polymerized vinyl esters (including copolymers of different esters), polymerized vinyl acetals, polymerized vinylidene esters, copolymers of vinyl and vinylidene esters, polystyrene, polyvinyl naphthalene, cellulose esters, ethyl cellulose, sulphurized vegetable oils (factice), polyisobutylene, and the various water-insoluble synthetic resins which are the so-called synthetic rubber or rubber-like materials, namely, butadiene polymers (polymerized butadiene-1,3, chloro-2-butadiene-1,3 ("neoprene"), methyl-2-butadiene-1,3, 2,3-dimethyl butadiene-1,3), copolymers of a major proportion of a butadiene and a minor proportion of a monovinyl compound copolymerizable therewith such as styrene ("Buna S") or acrylic nitrile ("Buna N"), copolymers of a major proportion of isobutylene and a minor proportion of a diolefine copolymerizable therewith such as butadiene-1,3 or 2-methyl butadiene-1,3 (isoprene), or 2,3-dimethyl butadiene-1,3 or pentadiene-1,3 ("Butyl" rubbers), organic polysulphide polymer plastics (commercially known as "Thiokols" and which are substantially polymers of the structural unit



or the structural unit



where



represents two carbon atoms separated by and joined to an intervening structure such as an ether linkage, unsaturated carbon atoms, aromatic structure, saturated straight chain hydrocarbons, or saturated branch chain hydrocarbons as described in the Patrick Patents Nos. 1,890,191 and 2,216,044, respectively.

In carrying out the process of the invention, the fabric is immersed in a bath of an agglomerated water-insoluble resin composition as described above, until the desired amount of resin flocs has deposited on the fabric, after which the fabric may be rinsed or washed, and dried. The fabrics may be woven or knitted and may be made of various kinds of fibers, such as silk, wool, cotton, linen, viscose rayon, acetate rayon, cuprammonium rayon, synthetic fibers such as nylon, and the like, or various combinations of the same. The process of the present invention is particularly adapted to the treatment of knitted fabrics, such as stockings, where the treatment imparts to the stockings an appearance of having been knit from finer yarns or on finer gauge machines in addition to enhancing the wearing qualities and reducing the tendency to snag.

The fabric, according to the present invention, is immersed in a bath where the weight ratio of treating bath to fabric ranges from 10:1 to 80:1, or over, and the fabric is permitted to remain in the bath until the desired amount of flocs is deposited on the fabric. Small amounts of acid or alkali may be added to the bath during the deposition treatment depending on the method used in agglomerating the resin particles. For

example, if the resin particles have been flocculated by addition of an acid salt such as ammonium sulphate, small amounts of acid may be added during the deposition, and if the resin particles have been flocculated by addition of an alkaline salt, such as sodium carbonate, small amounts of alkaline material may be added during the deposition. The treating bath may contain up to 2% water-insoluble synthetic resin and where weight ratio of bath to fabric is not too high, all of the flocculated resin particles may be deposited. The ratio of treating bath to fabric and the concentration of resin in the bath determine the amount of resin deposit on the fabric. The bath of resin agglomerates may be acid, neutral, or alkaline, depending on the method of agglomerating the resin particles from the dispersed state and the type of resin dispersion employed. The resin agglomerates are firmly anchored or set on deposition. The fabric with the resin deposit thereon may be washed or rinsed in plain water before drying. However, the pH of the rinse water is preferably similar to that of the treating bath at the end of the deposition so as to prevent any tendency for the resin agglomerates to be washed out or discharged in the rinsing operation before drying.

Various examples of the treatment of fabrics are set forth below, but these are merely exemplary of the invention and are not intended to be limitations thereof.

#### Example I

In this case rayon stockings were treated with 35 a methacrylate resin. The starting material was a commercial emulsion supplied by E. I. du Pont de Nemours & Co., under the trade name "Methacrylate-NH Emulsion," which is an aqueous dispersion of polymerized methyl methacrylate.

In making up the treating bath from the 40 "Methacrylate-NH Emulsion," 16 lbs. of water were placed in a stainless steel container at 110° F. 3 ounces of a 5% aqueous solution of Aquarex D, a stabilizer having the composition 45 mono sodium sulphate ester of one-half lauryl and one-half myristyl alcohol, were added, and then, in order, were added 1 oz. of "Methacrylate-NH Emulsion" containing 40% resin, 1 oz. of a 40% aqueous clay dispersion and 5 oz. of 3% aqueous gelatin solution. The bath was well stirred and 3 lbs. of 33 1/3% aqueous solution of ammonium sulphate were added. On addition of the ammonium sulphate, the dispersed particles in the bath immediately agglomerated and on removing a portion of the bath from the container in a graduate for inspection, the flocs could be seen to settle immediately.

A dozen pairs of all-rayon full-fashioned ladies' 60 stockings which weighed one pound, were introduced into a cotton bag and placed into the bath. The stockings were agitated in the bath and after 10 minutes, 1 1/4 oz. of 10% formic acid were added, followed by 2 1/2 oz. of the 10% formic acid solution after 10 more minutes, and again 2 1/2 oz. more after 10 more minutes. At the end of 15 more minutes, or 45 minutes total treatment, the stockings in the cotton bag were removed. The bath was clear. The stockings were rinsed in fresh water, removed, the excess water extracted in a centrifuge, and the stockings dried on heated forms in the usual manner. The stockings were found to have gained 3% in weight, the balance of the resin having deposited upon the cotton bag. The hosiery had

a very sheer appearance and had improved resistance to bagging, snagging and wear.

*Example II*

In this case stockings were treated with a flocculated "Nypene Emulsion 1802" supplied by The Neville Company. This was an aqueous dispersion of a polyterpene resin made by the catalytic polymerization of turpentine.

In preparing the treating bath, 92 lbs. of water were introduced into the stainless steel container, followed by 6 oz. of a 5% solution of Aquarex D, 2 oz. of a 40% emulsion of "Nypene Emulsion 1802," 2 oz. of a 40% aqueous clay dispersion, and 10 oz. of a 3% gelatin solution. 6 lbs. of a 33 1/3% aqueous solution of ammonium sulphate were added and the material in the bath flocculated immediately.

Two dozen pairs of ladies stockings with rayon legs and cotton plated feet weighing 2 lbs. were introduced into the bath and agitated therein, and after 10 minutes 2 1/2 oz. of aqueous 10% formic acid was added, followed by 5 oz. of the formic acid solution after 10 minutes, and 5 oz. again after 10 more minutes. The stockings were removed from the bath after 45 minutes from the time of initial immersion. The bath was clear and the stockings were found to have gained 3.2% in weight. The stockings showed marked improvement in appearance and wearing qualities.

*Example III*

In this case the fabric was treated with polyvinyl acetate resin. The starting material was polyvinyl acetate emulsion "RH 460 A" supplied by E. I. du Pont de Nemours & Co., which is an aqueous dispersion of polyvinyl acetate resin. The emulsion contained 40% of the resin.

The treating bath was made up by introducing 155 lbs. of water into a stainless steel container and adding thereto 1 lb. of 5% aqueous solution of Aquarex D, 5 oz. of the 40% "RH-460 A" polyvinyl acetate resin, 5 oz. of the 40% aqueous clay dispersion, and 1.5 oz. of the 3% gelatin solution. The bath was then flocculated by adding thereto 15 pounds of a 33 1/3% aqueous solution of ammonium sulphate.

Four dozen pairs of cotton-top rayon stockings weighing 5 lbs. were introduced into the bath in the usual cotton bag, and after 10 minutes of agitating, 6 oz. of 10% aqueous solution of formic acid was added, followed by 12 oz. of the 10% formic acid after 10 more minutes, and then 12 oz. again after a further 10 minutes. The stockings were removed from the bath 45 minutes after initial immersion and the bath was clear. The gain in weight on the stockings was found to be 4%. Marked improvement in appearance and wearing qualities of the stockings was noted.

*Example IV*

In this case stockings were treated with polymerized butyl methacrylate.

The butyl methacrylate polymer dispersion was prepared by plasticizing 100 parts of the commercial polymer with 50 parts of butyl benzyl sulphonamide, milling in 20 parts of alkali-solubilized casein as a dispersing agent, and then adding water slowly in a Werner & Pfeiderer mixer until an inversion in phase took place and the resin became dispersed in the aqueous medium, and adding further water to a concentration of 50% solids (all parts designated herein are by weight). To the 340 parts of the disper-

sion of the butyl methacrylate polymer was added 105 parts of a 24-hour ball-milled aqueous clay dispersion containing 50 parts of Dixie clay and 5 parts of "Aquarex D," 1200 parts of a 3% gelatin solution, and 560 parts water.

A flocculated treating bath was prepared in which the ratio of bath to stockings was 20:1. The bath contained 50 parts of the above dispersion of the butyl methacrylate and clay, 150 parts of a 33 1/3% solution of ammonium sulphate, and 25 parts of a 10% solution of "Aquarex D," per 100 parts of hosiery.

The stockings which were viscose rayon were introduced into the bath at 110° F., and after 5 minutes, 5 parts of 10% aqueous formic acid per 100 parts of hosiery were added, followed by 10 parts of 10% formic acid after 5 more minutes, and then 10 parts of 10% formic acid after a further 5 minutes. The stockings were removed from the bath after 30 minutes. The bath which was slightly hazy was discarded. The stockings were rinsed twice at 110° F. in 20:1 rinse baths containing 50 parts of 10% formic acid per 100 parts of hosiery, extracted, and dried. The gain in weight on the stockings was 3.3%.

*Example V*

In this case stockings were treated with "Vinsol Plastic," which is a copolymer of Vinsol (the 30 still residuum after the distillation of turpentine) and fish oil.

The Vinsol Plastic dispersion was prepared by compounding 100 parts of the commercial Vinsol Plastic with 4 parts of sulphur and 10 parts of 35 zinc oxide, milling in 1 part of alkali-solubilized casein and 8 parts of dimethylamine soap as dispersing agents, and then adding water slowly in a Werner & Pfeiderer mixer until an inversion of phase took place and the plastic became dispersed in the aqueous medium, and adding further water to a concentration of 50% solids. To the 246 parts of the dispersion of the Vinsol Plastic was added 105 parts of a 24-hour ball-milled aqueous clay dispersion containing 50 parts of Dixie clay and 5 parts of "Aquarex D," 1200 parts of a 3% gelatin solution, and 100 parts of water.

A flocculated treating bath was prepared in which the ratio of bath to stockings was 20:1. The bath contained 45 parts of the above dispersion of the Vinsol Plastic and clay, 27 parts of a 10% solution of "Aquarex D," and 150 parts of 33 1/3% solution of ammonium sulphate, per 100 parts of hosiery.

The stockings which were viscose rayon were introduced into the bath at 110° F. and after 10 minutes 5 parts of 10% formic acid per 100 parts of hosiery were added, followed by 10 parts of 10% formic acid after 10 more minutes, and then 10 parts of 10% formic acid after a further 10 minutes. The stockings were removed from the bath after 45 minutes. The bath which was slightly hazy was discarded. The stockings were rinsed twice at 110° F. in 20:1 rinse baths containing 50 parts of 10% formic acid per 100 parts of hosiery, extracted, and dried. The gain in weight on the stockings was 3.5%.

*Example VI*

In this case viscose rayon stockings were treated with commercial polyvinyl butyral.

The polyvinyl butyral as obtained contained 7 parts of a plasticizer per 100 parts of the polyvinyl butyral resin. The dispersion was prepared by plasticizing 107 parts of the polyvinyl resin

as received with 50 parts of castor oil, milling in 15 parts of ammonium soap, and then adding water slowly in a Werner & Pfleiderer mixer until an inversion of phase took place and the resin became dispersed in the aqueous medium, and adding further water to a concentration of 55% solids. To the 312 parts of the dispersion of the polyvinyl butyral was added 105 parts of a 24-hour ball-milled aqueous dispersion containing 50 parts of Dixie clay and 5 parts of "Aquarex D," and 1200 parts of a 3% gelatin solution.

A flocculated treating bath was prepared in which the ratio of bath to stockings was 40:1. The bath contained 38 parts of the above polyvinyl butyral and clay dispersion, 300 parts of a 33½% solution of ammonium sulphate, and 25 parts of a 10% solution of "Aquarex D," and 1 part of a 10% formic acid solution, per 100 parts of hosiery.

The stockings were introduced into the bath at 110° F. and after 15 minutes and again after 15 more minutes, 1.5 parts of 10% formic acid per 100 parts of hosiery were added. The stockings were removed from the bath after 45 minutes. The bath which was slightly hazy was discarded. The stockings were rinsed twice in 40:1 rinse baths containing 1 part of 10% formic acid per 100 parts of hosiery, extracted, and dried. The gain in weight on the stockings was 1.7%.

#### Example VII

In this case viscose rayon stockings were treated with a flocculated dispersion of a phenol-formaldehyde resin. The starting material was a commercial aqueous phenol-formaldehyde dispersion—"Durez Emulsion No. 2-9230," supplied by the Durez Plastics & Chemical Inc. The dispersion contained 50% solids.

To 100 parts of the dispersion of the phenol-formaldehyde resin was added 105 parts of a 24-hour ball-milled dispersion containing 50 parts of Dixie clay, and 5 parts of "Aquarex D."

A flocculated treating bath was prepared in which the ratio of bath to stockings to be treated was 40:1. The bath contained 12 parts of the above phenol-formaldehyde and clay dispersion, 150 parts of a 33½% solution of ammonium sulphate, 25 parts of a 10% solution of "Aquarex D," and 1 part of a 10% formic acid solution, per 100 parts of hosiery.

The stockings were introduced into the bath at 110° F. and after 15 minutes and again after 15 more minutes 1.5 parts of 10% formic acid solution per 100 parts of hosiery were added. The stockings were removed from the bath after 45 minutes. The bath which was slightly hazy was discarded. The stockings were rinsed twice in 40:1 rinse baths containing 1 part of a 10% formic acid solution per 100 parts of hosiery, extracted, and dried. The gain in weight on the stockings was 3.4%.

#### Example VIII

In this case cuprammonium rayon stockings were treated with ethyl cellulose. The starting material was commercial ethyl cellulose supplied by Hercules Powder Company under the trade name "Ethocel."

The dispersion of ethyl cellulose was prepared by plasticizing 100 parts of the "Ethocel" with 25 parts of dibutyl phthalate, milling in 8 parts of diethylamine soap as a dispersing agent, and then adding water slowly in a Werner & Pfleiderer mixer until an inversion in phase took place and the "Ethocel" became dispersed in the

aqueous medium, and adding further water to a concentration of 10%.

A flocculated treating bath was prepared in which the ratio of bath to stockings was 35:1.

5 The bath contained 55 parts of the above ethyl cellulose dispersion, 25 parts of a 10% solution of the protective "Igepon T," 250 parts of a 33½% solution of ammonium sulphate, and 1 part of a 10% formic acid solution, per 100 parts of hosiery.

10 The stockings were introduced into the bath at 110° F. and after 15 minutes and again after 15 more minutes 1.5 parts of 10% formic acid per 100 parts of hosiery were added. The stockings were removed from the bath after 45 minutes. The bath which was slightly hazy was discarded. The stockings were rinsed twice in 35:1 rinse baths containing 2 parts of 10% formic acid per 100 parts of hosiery, extracted, and 15 dried. The gain in weight on the stockings was 3.2%.

#### Example IX

In this case viscose stockings were treated with commercial polyisobutylene furnished by 25 Standard Oil Company of New Jersey under the trade name "Vistanex."

The dispersion of polyisobutylene was prepared by milling in 20 parts of alkali solubilized casein and 2 parts of diethylamine soap per 30 100 parts of polyisobutylene as dispersing agents, and then adding water slowly in a Werner & Pfleiderer mixer until an inversion of phase took place and the resin became dispersed in the aqueous medium, and adding further water 35 to a concentration of 50% solids.

To 244 parts of the isobutylene dispersion was added 105 parts of a 24-hour ball-milled dispersion containing 50 parts of Dixie clay and 5 parts of "Aquarex D," 1200 parts of a 3% gelatine solution, and 100 parts of water.

A flocculated treating bath was prepared in which the ratio of bath to stockings was 20:1. The bath contained 45 parts of the above polyisobutylene and clay dispersion, 12 parts of a 10% solution of "Aquarex D" and 150 parts of a 33½% solution of ammonium sulphate, per 100 parts of hosiery.

The stockings were introduced into the bath at 110° F. and after 10 minutes 1 part of 10% aqueous formic acid per 100 parts of hosiery was added, followed by 2 parts of 10% of formic acid after 5 more minutes, and then 2 parts of 10% formic acid after a further 5 minutes. The stockings were removed from the bath after 40 minutes. The bath which was slightly hazy was discarded. The stockings were rinsed once at 110° F. in a 20:1 rinse bath containing 5 parts of 10% formic acid per 100 parts of hosiery, extracted, and dried. The gain in weight on the hosiery was 2.7%.

#### Example X

In this case viscose rayon stockings were treated with a polyhydric alcohol-polybasic acid polymer—"Noropol" made by the condensation polymerization of so-called soy bean acid and ethylene glycol.

10 70 75 100 parts of the Noropol were first compounded with 25 parts ester gum, 50 parts zinc oxide, 5 parts sulphur and 2 parts mercaptobenzothiazole (accelerator), and the compound cured or vulcanized by heating for 3 hours at 150° C. The 182 parts of the cured Noropol were dispersed in a Werner & Pfleiderer mixer on 36

parts of gelatin with addition of water to a 50% solids dispersion in the conventional manner.

A flocculated treating bath was prepared in which the ratio of bath to stockings was 20:1. The bath contained 10 parts of the 50% solids dispersion of the Noropol, 25 parts of 10% solution of "Aquarex D," 150 parts of a 33½% solution of ammonium sulphate, and 1 part of 10% formic acid solution, per 100 parts of hosiery.

The stockings were introduced into the bath at 110° F. and after 15 minutes and again after 15 more minutes 1.5 parts of 10% formic acid per 100 parts of hosiery were added. The stockings were removed from the bath after 45 minutes. The bath which was clear was discarded. The stockings were rinsed twice in a 20:1 rinse bath containing 2 parts of 10% formic acid per 100 parts of hosiery, extracted, and dried. The gain in weight on the stockings was 8.2%.

#### Example XI

In this case viscose rayon stockings were treated with a flocculated dispersion of Noropol dispersed on gelatin which also acted as the protective to prevent lump coagulation of the dispersion on flocculation.

A flocculated treating bath was prepared in which the ratio of bath to stockings was 20:1. The Noropol dispersion used was the same 50% solids dispersion as in Example X in which 182 parts of the cured Noropol was dispersed on 36 parts of gelatin. The bath contained 6½ parts of the 50% Noropol dispersion per 100 parts of hosiery and 3½ parts of a 24-hour ball-milled 40% dispersion of Dixie clay containing .8% gelatin. The bath was flocculated by the addition of 10 parts of a 5% aqueous solution of sodium carbonate, per 100 parts of hosiery.

The stockings were introduced into the bath at 110° F. and after 5 minutes 1 part of 10% aqueous ammonia per 100 parts of hosiery was added, followed by 2 parts of 10% ammonia after 5 more minutes, and then 2 parts of 10% ammonia after a further 5 minutes. The stockings were removed from the bath after 20 minutes. The bath which was slightly hazy was discarded. The stockings were rinsed once at 110° F. for 5 minutes in a 20:1 rinse bath containing 5 parts of 10% ammonia per 100 parts of hosiery, extracted, and dried. The gain in weight on the stockings was 2.7%.

#### Example XII

In this case viscose rayon stockings were treated with a Noropol dispersion dispersed on a cationic soap which also acted as the protective to prevent lump coagulation of the dispersion on flocculation.

A flocculated treating bath was prepared in which the ratio of bath to stockings was 20:1. 100 parts of the Noropol were first compounded with 25 parts of ester gum, 50 parts zinc oxide, 5 parts sulphur and 2 parts mercaptobenzothiazole (accelerator), and the compound cured or vulcanized by heating for 3 hours at 150° C. The 182 parts of the cured Noropol were dispersed in a Werner & Pfleiderer mixer by mixing in 36½ parts of a cationic base, mu-heptadecyl-N-hydroxyethyl imidazoline, and 6½ parts of glacial acetic acid to saponify the cationic base in situ and form the cationic soap, followed by the gradual addition of 225 parts of water to give a 50% solids dispersion.

A flocculated treating bath was prepared in which the ratio of bath to stockings was 20:1.

The bath contained 6½ parts of the 50% Noropol dispersion per 100 parts of hosiery, and 3½ parts of a 24-hour ball-milled 40% dispersion of Dixie clay containing .7% of acetic acid saponified mu-heptadecyl-N-hydroxyethyl imidazoline. The bath was flocculated by the addition of 10 parts of a 5% aqueous solution of sodium carbonate per 100 parts of hosiery.

The stockings were introduced into the bath at 110° F. and after 5 minutes 1 part of 10% aqueous ammonia per 100 parts of hosiery was added, followed by another 1 part of 10% ammonia after 5 more minutes, and then 1 part of 10% ammonia after a further 5 minutes. The stockings were removed from the bath after 20 minutes. The bath which was slightly hazy was discarded. The stockings were rinsed once at 110° F. for 5 minutes in a 20:1 rinse bath containing 2 parts of 10% ammonia per 100 parts of hosiery, extracted, and dried. The gain in weight on the stockings was 4.2%.

#### Example XIII

In this case cellulose acetate rayon stockings were treated with factice. The starting material 25 was a commercial dispersion of white factice of 40% solids content supplied by Stamford Rubber Supply Company.

A flocculated treating bath was prepared in which the ratio of stockings to bath was 30:1. 30 The bath contained 15 parts of the factice dispersion, 25 parts of a 10% solution of a commercial liquid stabilizer of unknown composition, sold by E. I. du Pont de Nemours & Co. under the trade name "MP-189-S Crude," and which as stated 35 by them to be a sulphonated petroleum product made to replace "Aquarex D," 250 parts of 33½% solution of ammonium sulphate, and 1 part of a 10% solution of formic acid per 100 parts of hosiery.

40 The stockings were introduced into the bath at 110° F., after 15 minutes and again after 15 more minutes 1.5 parts of 10% formic acid per 100 parts of hosiery were added. The stockings were removed from the bath after 45 minutes. The 45 bath was discarded, and the stockings were rinsed twice in 35:1 rinse baths containing 2 parts of 10% formic acid per 100 parts of hosiery, extracted, and dried. The gain in weight on the stockings was 2.4%.

#### Example XIV

In this case viscose rayon stockings were treated with a butadiene polymer, namely polymerized chloro-2-butadiene-1,3, known as neoprene. The 55 starting material was "Neoprene No. 571 Latex" which is a 50% dispersion of polychloroprene supplied by E. I. du Pont de Nemours & Co.

To 200 parts of the neoprene dispersion was added 125 parts of a 10% solution of "Aquarex D," 1200 parts of a 3% solution of gelatin, and 105 parts of a 24-hour ball-milled aqueous dispersion containing 50 parts of Dixie clay and 5 parts of "Aquarex D," and 280 parts of water.

A flocculated treating bath was prepared in 65 which the ratio of bath to stockings was 20:1. The bath contained 50 parts of the above dispersion of neoprene and clay, 35 parts of a 10% solution of "Aquarex D," and 150 parts of 33½% solution of ammonium sulphate, per 100 parts of hosiery.

70 The stockings were introduced into the bath at 110° F. and after 5 minutes 1 part of a 10% formic acid per 100 parts of hosiery was added, followed by 2 parts of a 10% aqueous formic acid after 5 more minutes, and then 2 parts of

10% formic acid after a further 5 minutes. The stockings were removed from the bath after 20 minutes. The bath which was slightly hazy was discarded. The stockings were rinsed for 10 minutes at 110° F. in a 20:1 rinse bath containing 3.5 parts of 10% formic acid per 100 parts of hosiery, extracted, and dried. The gain in weight on the stockings was 2.5%.

*Example XV*

In this case stockings were treated with a copolymer of butadiene and styrene, known as "Buna S." The starting material was the product of the emulsion-copolymerization of 75 parts butadiene-1,3 and 25 parts by weight of styrene in the presence of suitable protectives. To the dispersion was added suitable vulcanizing ingredients. The prepared curing dispersion was a 36% solids content dispersion.

To 305 parts of the 36% Buna S dispersion was added 800 parts of a 3% gelatin solution, and 240 parts of water.

A flocculated treating bath was prepared in which the ratio of bath to stockings was 18:1. The bath contained 50 parts of the diluted Buna S dispersion containing the gelatin, 25 parts of a 10% solution of "Aquarex D," and 120 parts of a 33½% solution of ammonium sulphate, per 100 parts of hosiery.

The stockings which were viscose rayon were introduced into the bath at 110° F. and after 10 minutes 1 part of 10% aqueous formic acid was added per 100 parts of hosiery, followed by 2 parts of 10% formic acid after another 10 minutes, and then 2 parts of 10% formic acid after 10 more minutes. The stockings were removed from the bath after 40 minutes. The bath which was slightly hazy was discarded. The stockings were rinsed once at 110° F. in an 18:1 rinse bath containing 5 parts of 10% formic acid per 100 parts of hosiery, extracted, and dried. The gain in weight on the stockings was 2%.

This is a continuation-in-part of application Serial No. 428,050, filed January 24, 1942.

In view of the many changes and modifications that may be made without departing from the principles underlying the invention, reference should be made to the appended claims for an understanding of the scope of the protection afforded the invention.

Having thus described my invention, what I claim and desire to protect by Letters Patent is:

1. The process of treating fabrics which comprises immersing a fabric in an aqueous bath of an agglomerated aqueous dispersion of water-insoluble synthetic resin in which the resin agglomerates are macroscopic and readily separable from the aqueous medium on standing, the weight ratio of said bath to said fabric being between 10:1 and 80:1 and said bath being capable of depositing its resin agglomerates on said fabric on contact therewith, and maintaining said fabric associated with said bath until the desired amount of flocculated resin particles has deposited on the fabric.

2. The process of treating fabrics which comprises immersing a fabric in an aqueous bath of an agglomerated dispersion of water-insoluble synthetic resin in which the resin agglomerates are in the form of composite particles comprising water-insoluble synthetic resin and clay which are macroscopic and readily separable as such composite particles from the aqueous medium on standing, the weight ratio of said bath to said fabric being between 10:1 and 80:1 and said bath

being capable of depositing its resin agglomerates on said fabric on contact therewith, and maintaining said fabric associated with said bath until the desired amount of composite particles has deposited on the fabric.

3. The process of treating fabrics which comprises immersing a fabric in an aqueous bath of an agglomerated aqueous dispersion of water-insoluble synthetic resin in which the resin agglomerates are macroscopic and readily separable from the aqueous medium on standing, the weight ratio of said bath to said fabric being between 10:1 and 80:1 and said bath containing sufficient protective to prevent the resin agglomerates from completely coagulating into a coherent lump but insufficient protective to prevent the agglomerates from depositing on the fabric, and maintaining said fabric associated with said bath until the desired amount of flocculated resin particles has deposited on the fabric.

4. The process of treating fabrics which comprises immersing a fabric in an aqueous bath of an agglomerated dispersion of water-insoluble synthetic resin in which the resin agglomerates are in the form of composite particles comprising water-insoluble synthetic resin and clay which are macroscopic and readily separable as such composite particles from the aqueous medium on standing, the weight ratio of said bath to said fabric being between 10:1 and 80:1 and said bath containing sufficient protective to prevent the resin agglomerates from completely coagulating into a coherent lump but insufficient protective to prevent the agglomerates from depositing on the fabric, and maintaining said fabric associated with said bath until the desired amount of composite particles has deposited on the fabric.

5. The process of treating fabrics which comprises immersing a fabric in an aqueous bath of an agglomerated aqueous dispersion of water-insoluble synthetic resin in which the resin agglomerates are macroscopic, said bath being capable of depositing its resin aggregates on said fabric on contact therewith, and maintaining said fabric associated with said bath until the desired amount of flocculated resin particles has deposited on the fabric.

6. The process of treating fabrics which comprises immersing a fabric in an aqueous bath of an agglomerated aqueous dispersion of water-insoluble synthetic resin in which the resin agglomerates are macroscopic, said bath containing sufficient protective to prevent the resin agglomerates from completely coagulating into a coherent lump but insufficient protective to prevent the agglomerates from depositing on the fabric, and maintaining said fabric associated with said bath until the desired amount of flocculated resin particles has deposited on said fabric.

7. The process of treating fabrics which comprises immersing a fabric in an aqueous bath of an agglomerated aqueous dispersion of water-insoluble synthetic resin containing up to 2% water-insoluble synthetic resin and in which the resin particles are macroscopic and readily separable from the aqueous medium on standing, the weight ratio of said bath to said fabric being between 10:1 and 80:1, and said bath being capable of depositing its resin agglomerates on said fabric on contact therewith, and maintaining said fabric associated with said bath until the desired amount of flocculated resin particles has deposited on the fabric.

8. The process of treating fabrics which com-

prises immersing a fabric in an aqueous bath of an agglomerated dispersion of water-insoluble synthetic resin containing up to 2% water-insoluble synthetic resin and in which the resin agglomerates are in the form of composite particles comprising water-insoluble synthetic resin and clay which are macroscopic and readily separable as such composite particles from the aqueous medium on standing, the weight ratio of said bath to said fabric being between 10:1 and 80:1 and said bath being capable of depositing its resin agglomerates on said fabric on contact therewith, and maintaining said fabric associated with said bath until the desired amount of composite particles has deposited on the fabric.

9. The process of treating fabrics which comprises immersing a fabric in an aqueous bath of an agglomerated aqueous dispersion of water-insoluble synthetic resin containing up to 2% water-insoluble synthetic resin and in which the resin agglomerates are macroscopic and readily separable from the aqueous medium on standing, the weight ratio of said bath to said fabric being between 10:1 and 80:1 and said bath containing sufficient protective to prevent the resin agglomerates from completely coagulating into a coherent lump but insufficient protective to prevent the agglomerates from depositing on the fabric, and maintaining said fabric associated with said bath until the desired amount of flocculated resin particles has deposited on the fabric.

10. The process of treating fabrics which comprises immersing a fabric in an aqueous bath of an agglomerated dispersion of water-insoluble synthetic resin containing up to 2% water-insoluble synthetic resin and in which the resin agglomerates are in the form of composite particles comprising water-insoluble synthetic resin

and clay which are macroscopic and readily separable as such composite particles from the aqueous medium on standing, the weight ratio of said bath to said fabric being between 10:1 and 80:1 and said bath containing sufficient protective to prevent the resin agglomerates from completely coagulating into a coherent lump but insufficient protective to prevent the agglomerates from depositing on the fabric, and maintaining said fabric associated with said bath until the desired amount of composite particles has deposited on the fabric.

11. The process of treating fabrics which comprises immersing a fabric in an aqueous bath of an agglomerated aqueous dispersion of water-insoluble synthetic resin containing up to 2% water-insoluble synthetic resin and in which the resin agglomerates are macroscopic, said bath being capable of depositing its resin aggregates on said fabric on contact therewith, and maintaining said fabric associated with said bath until the desired amount of flocculated resin particles has deposited on the fabric.

12. The process of treating fabrics which comprises immersing a fabric in an aqueous bath of an agglomerated aqueous dispersion of water-insoluble synthetic resin containing up to 2% water-insoluble synthetic resin and in which the resin agglomerates are macroscopic, said bath containing sufficient protective to prevent the resin agglomerates from completely coagulating into a coherent lump but insufficient protective to prevent the agglomerates from depositing on the fabric, and maintaining said fabric associated with said bath until the desired amount of flocculated resin particles has deposited on said fabric.

HOWARD A. YOUNG.